

Nov. 14, 1961

D. R. ALLEN ET AL

3,008,881

## PRODUCTION OF URANIUM

Filed June 30, 1958



Fig. 2



Fig. 1

*64* INVENTORS.  
*Donald R. Allen*  
*Anneke S. Allen*

BY C. W. Carlin.

**ATTORNEY**

1

3,008,881

## PRODUCTION OF URANIUM

Donald R. Allen and Anneke S. Allen, Lake Jackson, Tex., assignors to The Dow Chemical Company, Midland, Mich., a corporation of Delaware

Filed June 30, 1958, Ser. No. 745,716  
3 Claims. (Cl. 204—1.5)

The invention is directed toward a method of producing uranium metal electrolytically and toward an improved cell and electrolyte employed in such method.

The increased demand for uranium due to its importance in the study of nuclear principles and in the application of these principles has accentuated the need for more efficient and more economical methods of and means for producing uranium.

Methods currently employed in the production of uranium include the preparation of  $UF_4$  from uranium oxide, extracted from ore containing commercial quantities of such oxides, and reducing the  $UF_4$  by the action of calcium or magnesium metal to metallic uranium wherein one mole of the uranium metal to two moles of the  $CaF_2$  or  $MgF_2$  is produced. Methods currently employed also include the production of uranium metal electrolytically in which either  $KUF_5$  or  $UF_4$  is dissolved in a fused salt bath consisting essentially of a major proportion of  $CaCl_2$  and a minor proportion of  $NaCl$  to comprise the electrolyte which is electrolyzed in a graphite crucible at a temperature of about  $900^\circ C$ . The crucible serves as the anode and a high melting metal, e.g., Mo, somewhat centrally located, serves as the cathode upon which the uranium metal deposits during the electrolytic process.

These methods do not meet all the requirements for large-scale low-cost production of uranium metal.  $UF_4$  is an undesirable intermediate since it is corrosive and presents certain health hazards. The  $UF_4$  salt must meet rigid specifications: it should be substantially anhydrous and free of contaminants and of a particle size such that about 86 to 99 percent passes through a number 60 U.S. Standard sieve and 52 to 62 percent of it passes through a number 325 sieve. Furthermore, the employment of known salt baths in electrolytic cells of known structure has not resulted in a satisfactory electrolysis of the uranium salt.

A need, therefore, exists for better ways and means for producing uranium metal. Accordingly, the fundamental objects of the invention are to provide an improved method of producing uranium metal and to provide a novel electrolyte and electrolytic cell for use in such method.

The accomplishment of the foregoing and related objects by the practice of the invention, as hereinafter fully described in reference to the annexed drawing and particularly pointed out in the appended claims, consists of an improved electrolyte, electrolytic cell, and method of producing uranium metal by recovering it at the cathode of an electrolytic cell provided with an alkali metal anode suspended or floated on an electrolyte consisting of a mixture of an alkali metal chloride and an alkali metal uranous fluoride at a temperature above the melting point of the electrolyte. The temperature of the electrolyte should not be substantially above its melting point because an unnecessarily high temperature tends to raise the temperature of the exposed portion of the alkali metal anode above its vaporization point.

The anode can be molten potassium, sodium or lithium, but is usually sodium. It is contained in an elongated substantially vertical holder having an open lower end and having any desired cross-sectional shape, cylindrical being the most practical. The vertical holder can be of any material which has a sufficiently high melting point

2

and is unreactive with both the anode material and the electrolyte. It is preferably an electrical conductor such as carbon, graphite, molybdenum, tantalum, or tungsten, or uranium or molybdenum-clad steel so that the electrical connection may be made to it. However, the electrical connection may be made to the alkali metal directly in which case the holder may be either a conductor or non-conductor of electricity.

Some of the alkali metal in the vertical holder tends to volatilize when the height of the column of metal in the holder is low. This condition can be overcome either by providing a cover for the upper end of the anode holder or for the entire top of the electrolyte chamber and maintaining an inert gas in the zone above the alkali metal and/or by maintaining the alkali metal column of sufficient height to result in a temperature at the top of the column which is substantially lower than the vaporization temperature of the alkali metal and to provide a hydrostatic head to discourage volatilization of the alkali metal in contact with the electrolyte. The holder for the alkali metal should be sufficiently long to provide a zone above the metal for condensation of any alkali metal vapors formed and to extend sufficiently far beneath the surface of the electrolyte to permit a sufficiently high column of alkali metal for the desired hydrostatic head. The metal at the upper part of a column is at a desired height when it is below the vaporization temperature and thereby serves as a sort of cover.

$LiCl$ ,  $KCl$ , or  $NaCl$  may be used as the chloride in the electrolyte of the invention; however,  $NaCl$  is preferred.

The electrolyte may consist of a weight ratio of between 1 and 2 parts of the alkali metal uranous fluoride to one part of the alkali metal chloride but it is preferable that it be about 2 parts of the alkali metal uranous fluoride to 1 part of the alkali metal chloride. A percentage composition of about 65 percent of  $KUF_5$  or  $NaUF_5$  and about 35 percent  $NaCl$  is recommended. The temperature of the bath can be from  $650^\circ$  to  $850^\circ C$ , but it is preferred that it be from about  $750^\circ$  to  $800^\circ C$ . Only the alkali metal uranous fluoride enters into the electrolytic action. This is in contrast to known methods and cells for the production of uranium which employ mixtures containing an alkaline earth halide, usually a major proportion of such mixture being  $CaCl_2$ , which is a reactant during the electrolysis, forming  $CaF_2$ .

FIGURES 1 and 2 of the drawing illustrate the cell of the invention. FIGURE 1 is an elevational view largely in section taken at line 1—1 of FIGURE 2. FIGURE 2 is a horizontal section taken at line 2—2 of FIGURE 1.

Referring to the drawing in more detail there is shown electrolyte chamber 10 of electrically conducting material usually steel and consisting essentially of bottom 12 and cylindrical sidewall 14 about the upper edge of which is flange 16. Protective liner 17 covers the inside of bottom 12 and sidewall 14. It must be of an electrically conductive material substantially unreactive with uranium. Carbon or uranium is usually used. Liner 17 together with bottom 12 and sidewall 14 also serves as the cathode of the cell. Electrical heating coil 18 is positioned about sidewall 14 to heat chamber 10. Electrical lead-in lines 19 and 20 passing through electrically insulating ring-shaped gaskets 21 and 22, respectively, lead to a source of A.C. or D.C. to provide energy to the heating coil. Protective steel shell 23 incloses heating coil 18 and the bottom 12 of chamber 10. Electrically insulating spacers 24 help to support chamber 10 and provide free movement of heated air under bottom 12. Molten electrolyte 25 is shown partially filling chamber 10.

Electrically insulating gasket 26 is positioned on flange

16 which supports annular top plate 27. Cover 28 having top 29 and cylindrical sidewall 30 which has flange 31 at its lower edge is secured to gasket 26 and thence to plate 27 and flange 16 by means of bolts 32 which pass through aligned holes provided therefor in 31, 27, 26 and 16. Opening 33 in 27 equipped with cover 34 and opening 35 in 29 equipped with cover 36 provide access to the interior of the apparatus.

Upwardly extending neck 38 is shown centrally located in top plate 27. Supported substantially centrally in neck 38 by outwardly radiating arms 40 is open-end graphite anode tube 42. Tube 42 extends downwardly below the level of electrolyte 25 but does not reach bottom 12. Molten alkali metal 44 is shown floating on electrolyte 25 within tube 42.

Positive electrical lead-in line 46 passing through electrical insulating tightly fitting ring-shaped gasket 48 carries current to anode tube 42 from the positive terminal of a source of D.C. and line 50 passing through insulating tightly fitting ring-shaped gasket 52 carries current to sidewall 14 of chamber 10 from the negative terminal of the source of D.C.

Inlet line 54 having valve 56 therein provides a means for introducing an inert gas into the top of the cell. Line 58 having valve 60 therein provides a means for escape of gases from the top of chamber 10 of the cell.

In practicing the invention, a mixture of an alkali metal uranous fluoride and an alkali chloride, preferably  $\text{NaUF}_5$  and  $\text{NaCl}$ , in a weight ratio of about  $2\text{NaUF}_5$  to  $1\text{NaCl}$ , is placed in the electrolyte chamber and melted by means of a source of heat such as a gas furnace or electric heating coil shown in the drawing. An alkali metal, usually sodium, is placed in the anode holder where it becomes molten, as shown, and forms electrical contact with the electrolyte. The height of sodium metal in the holder is such that the sodium column, due to the hydrostatic head of the electrolyte, is a short distance above the open bottom end of the holder. Nitrogen gas is introduced through line 54 to blanket and protect the sodium from contamination or reaction with oxygen. The temperature of the electrolyte is maintained usually at from  $780^\circ$  to  $850^\circ$  C. In carrying out the electrolysis, only a relative low voltage is required. A voltage between 0.5 and about 10 volts can be used but a voltage between 1 and 2 volts is preferred. The electrode spacing is preferably close, on the order of about 1 inch. The current density based on the area of the alkali metal anode in contact with the electrolyte can be between 10 and 30 amperes/square inch, about 30 amperes/square inch usually being used.

As electrolysis proceeds, uranium metal accumulates at the bottom of the electrolyte chamber which serves as the cathode. The larger portion of the uranium metal collects on that part of the bottom of the cathode opposite the lower face of the anode. The alkali metal anode is gradually converted to alkali metal ions which enter the electrolyte, the alkali metal thereby gradually being consumed. When sodium is the alkali metal, the sodium ions are thought to react in the electrolyte according to the equation:



Sodium metal is, therefore, added periodically to tube 42 to replace the sodium thus used and  $\text{NaUF}$  is added to the electrolyte as required.

It might be thought that some chlorine or fluorine ions would be drawn to the positively charged alkali metal or holder therefor. However, there appears to be little evidence of this occurring to any appreciable extent. Such occurrence would be readily detected because the chlorine or fluorine ions thus drawn would react immediately with the sodium to form the sodium halide and would be measurable in the weight of sodium consumed per unit weight of uranium produced.

As desired, the uranium metal thus produced can be removed from the electrolyte by any convenient manner. It may be raked out during operation or the operation discontinued and while the electrolyte is molten, the electrolyte may be decanted off leaving the uranium metal and thereafter manually recovering the uranium metal; or the uranium can be removed by cooling the electrolyte to room temperature, removing the contents of the cell chamber, and thereafter separating the solid uranium from the electrolyte as by dissolving the electrolyte and recovering the uranium metal, e.g., by zone melting as described in AINE Transactions, volume 194, page 747 (1952), by W. G. Pfann.

Since, as stated, the uranium metal largely collects on that part of the cathode opposite the anode, a removable cathode plate or grid of unreactive conducting material, e.g., of uranium, may be placed opposite to the anode, periodically removed, and the accumulated uranium metal scraped therefrom.

Since the feed composition added to the cell before and/or during operation and the weight of alkali metal consumed are known, the bath composition may be readily calculated for the purposes of adding additional feed or stopping the operation according to the above equation.

The  $\text{NaF}$ , comprising the major portion of the separated electrolyte, can be used in a subsequent reaction to prepare double fluorides such as  $\text{NaTiF}_5$  or  $\text{NaSiF}_5$ , or to prepare more  $\text{NaUF}_5$  for further electrolysis according to the invention. For example, the latter can be prepared according to the following equation:



The following example illustrates the invention:

*Example*

An electrolytic cell of the type shown in the drawing was constructed and employed in the example. Covers 36 and 34 were removed and 300 grams of a salt mixture consisting by weight of 65 percent  $\text{NaUF}_5$  and 35 percent  $\text{NaCl}$  were placed in electrolyte chamber 10 of the cell through openings 35 and 33. Electric current was passed through heating coil 18 to heat the salt mixture. The salt mixture was melted thereby to form electrolyte 25 and the temperature thereafter was maintained at between  $780^\circ$  and  $800^\circ$  C. One hundred grams of metallic sodium were placed in tube 42 whereupon the sodium melted. Covers 34 and 36 were then replaced. Valves 56 and 58 were opened. Nitrogen gas was introduced through line 54 which flushed the air out vent 58. Valve 60 was then closed thereby blanketing the surface of the electrolyte and the sodium anode. Electric lines 46 and 50 were then connected to the positive and negative terminals, respectively, of a source of D.C. of between 1 and 2 volts which provided a flow of electricity through the electrolyte at between 45 and 50 amperes to effect electrolysis of the  $\text{NaUF}_5$ . The current density measured according to the area at the sodium anode exposed to the electrolyte was 30 amperes per square inch. As electrolysis proceeded, uranium metal accumulated at the bottom 12 of chamber 10. Because sodium metal 44 was gradually consumed during the electrolytic process, cover 36 was removed during electrolysis and 100 additional grams of sodium metal added to tube 42. The cell was operated for sixty-two minutes. The electric current was then shut off and the cell cooled to room temperature. Covers 36 and 34 were taken off and the uranium metal which had collected on bottom 12 of chamber 10 removed. 400,950 coulombs of electricity were used to produce 52 grams of 98 percent uranium.

It is to be understood that the above example is an illustration of but one mode of practicing the invention.

The method herein described, employing the electrolyte and the cell of the invention, represents a definite advancement in the art of uranium production. Here-

tofore, a consumable alkali metal anode has not been successfully employed in an electrolytic bath containing a compound of uranium. By practicing the invention, uranium metal may be produced at atmospheric pressure directly from a novel bath consisting of an alkali metal uranous fluoride and an alkali metal chloride which is readily prepared. Additional alkali metal uranous fluoride may be added to the electrolyte periodically, and the alkali metal chloride may be maintained more-or-less constant, during the electrolysis by merely adding additional alkali metal, e.g., sodium, to the anode. The need for further addition is determined by calculating the  $\text{NaUF}_5$  and Na metal used according to the equation set out hereinabove.  $\text{NaF}$  formed during electrolysis builds up in the electrolyte. By drawing off the excess electrolyte periodically, the  $\text{NaF}$  therein can be separated and thereafter conveniently employed to produce additional  $\text{NaUF}_5$  for use in the electrolyte of the invention.

Having described the invention, what is claimed and desired to be protected by Letters Patent is:

1. The method of producing uranium metal comprising electrolyzing a molten salt bath consisting essentially of at least 1 part by weight of an alkali metal uranous fluoride and not over 1 part by weight of an alkali metal chloride by passing D.C. between a cathode and an alkali metal anode in contact with the bath, said anode being substantially protected from contact with the air by a substantially unreactive gas, and recovering uranium metal at the cathode.

2. The method of producing uranium metal comprising passing D.C. between a negative electrode and a positive sodium metal electrode, substantially protected from con-

tact with the atmosphere by a substantially unreactive gas, said electrodes being in contact with a fused salt electrolyte consisting essentially of from about 60 to 70 percent  $\text{NaUF}_5$  and from about 40 to 30 percent  $\text{NaCl}$  5 by weight, recovering uranium metal at the cathode, and thereafter separating the uranium metal from the electrolyte.

3. A continuous method of producing uranium metal by floating a molten alkali metal on a molten salt electrolyte consisting essentially by weight of between 1 and 10 2 parts of an alkali metal uranous fluoride and 1 part of an alkali metal chloride confined in a conducting non-reactive container, said alkaline metal and molten salt electrolyte having a protective blanket of an inert gas 15 thereafter, making the alkali metal the anode and the conducting container the cathode, depositing said uranium metal on the floor of the container, adding additional alkali metal and alkali metal uranous fluoride, and removing the uranium metal thus deposited.

References Cited in the file of this patent

UNITED STATES PATENTS

|    |           |               |       |               |
|----|-----------|---------------|-------|---------------|
| 25 | 801,199   | Ashcroft      | ----- | Oct. 10, 1905 |
|    | 816,928   | Lyons et al.  | ----- | Apr. 3, 1906  |
|    | 2,512,206 | Holden et al. | ----- | June 20, 1950 |
|    | 2,598,833 | Reuman        | ----- | June 3, 1952  |
|    | 2,717,234 | Nagy et al.   | ----- | Sept. 6, 1955 |
|    | 2,752,303 | Cooper        | ----- | June 26, 1956 |
| 30 | 2,773,825 | Newcombe      | ----- | Dec. 11, 1956 |
|    | 2,773,826 | Beese et al.  | ----- | Dec. 11, 1956 |
|    | 2,774,729 | Meister       | ----- | Dec. 18, 1956 |